

Patented Sept. 8, 1936

2,053,821

# UNITED STATES PATENT OFFICE

2,053,821

## PROCESS FOR RETARDING THE ABSORPTION OF DYESTUFFS BY THE FIBER

Charles Graenacher, Basel, Franz Ackermann, Binningen, near Basel, Albert Landolt, Riehen, near Basel, and Wilhelm Geigy, Basel, Switzerland, assignors to Society of Chemical Industry in Basle, Basel, Switzerland

No Drawing. Application September 10, 1934, Serial No. 743,484. In Switzerland September 19, 1933

6 Claims. (Cl. 8—5)

According to this invention the absorption of dyestuffs by fibrous material is retarded by means of a dispersing agent containing, on the one hand, at least one basic nitrogen atom and at least one sulfo-group, which may be linked to a carbon atom or otherwise, e. g. to an oxygen atom, and, on the other hand, an aliphatic or cycloaliphatic radical containing at least 8 carbon atoms. By the expression "aliphatic or cycloaliphatic radical containing at least 8 carbon atoms" there are to be understood not only chains merely consisting of carbon atoms, but also chains which are interrupted by an oxygen-, sulfur- or nitrogen-bridge.

Examples of such dispersing agents are the sulfonic acids of cyclic amidines, such as are described in applications Serial No. 667,133 and No. 743,483, or obtained by sulfonation of the amidines described in the application Serial No. 727,584, as well as mixtures of such sulfonic acids.

If a water-soluble compound of this kind is added to a dye-bath the absorption of the dyestuff is very substantially retarded, so that in many cases there is a substantial improvement in the levelness of dyeings produced with the aid of such dyestuffs which would otherwise be rapidly absorbed. This effect can already occur in dyeing with basic dyestuffs cotton which has been mordanted with tannin or in some other suitable manner. The improvement in the levelling capacity may further be observed in the case of such direct-dyeing dyestuffs which are used for dyeing cellulosic fibers, such as cotton, artificial silk from regenerated cellulose, hemp, and ramie.

It is also clearly observed in the case of dyestuffs intended for dyeing animal fibers, such as wool or silk, particularly also in the case of acid dyestuffs which are rapidly absorbed, such as dyestuffs fast to milling, which must be dyed in an acetic acid bath. However, this effect is of particularly great practical importance in the case of alkaline baths containing hydrosulfite or other reducing agents having a similar action, and dyestuffs capable of being dyed in the reduced state, such as sulfur- or vat-dyestuffs, particularly vat-dyestuffs of the anthraquinone series being rapidly absorbed by the fibers. The retardation of the absorption capacity results, on the one hand, in an improvement of the levelness of the dyeings obtained, and, on the other hand, in an increase in the capacity for alkaline reducing baths to strip dyeings produced with vat-dyestuffs. Thus whilst many vat-dyestuff dyeings are scarcely affected by alkaline reducing baths, the addition to the bath of a compound used in accordance with the invention has the result that the dyeings undergo a pronounced weakening which renders it possible to improve the levelness of unlevel defective vat-dyeings. When used in dye-baths containing reducing agents those

among the above cited products have proved particularly effective which contain such sulfonated benzimidazole derivatives which are substituted at the  $\mu$ -carbon atom or at the N-atom by a longer aliphatic chain which may be interrupted. Among these, as is the case quite generally, the monosulfonic acids are particularly valuable. Further such sulfonic acids in which the longer chain is to be found at the  $\mu$ -carbon atom, and in which one or the two N-atoms are alkylated. Also sulfonation products of the mixture of mono-alkylated benzimidazoles and quaternary benzimidazolium compounds which are substituted at the  $\mu$ -carbon atom are particularly valuable. Particularly favorable results are obtained with compounds in which the N-alkyl radicals do not contain more than 4 carbon atoms. Consequently, the alkaline baths which, besides the reducing agents, contain the above characterized sulfonic acids, particularly the sulfonated imidazoles, represent valuable new agents which are used both for dyeing vat dyestuffs and for stripping textile materials dyed with vat-dyestuffs.

The following examples illustrate the invention:—

### Example 1

There is added to the dye-bath, containing 0.5 per cent. of trichloroisodibenzanthrone, vatted in the usual manner in an alkaline hydrosulfite bath, the sulfonated cyclic amidine, obtained by sulfonation of N-methyl- $\mu$ -heptadecylbenzimidazole, in quantity amounting to 0.25 gram per liter of dye-bath. The absorption of the dyestuff from the bath is appreciably retarded, so that the dyeings obtained are more level and the material is better through-dyed than is the case in the absence of the sulfonated amidine. The N-alkyl, N-propyl or N-butyl- $\mu$ -heptadecylbenzimidazole sulfonic acids behave quite similarly.

### Example 2

A material which has been dyed with 1.5 per cent. of Cibanone Blue 3G (Schultz, Farbstofftabellen No. 1,279) but which is defective owing to unlevelness, is treated for half-an-hour at 60° C. in a bath, containing per liter, 16 cc. of an aqueous solution of sodium hydroxide of 35° Bé. and 2 grams of sodium hydrosulfite. By the addition of 1 gram per liter of the sulfonated cyclic amidine, prepared by sulfonation of the mixture of N-methylated imidazoles from ortho-phenylenediamine and hydrogenated fish oil, the reabsorption of the reduced dyestuff which has been removed is retarded, whereby the dyeing is levelled. The product may also be used for stripping vat-dyeings.

### Example 3

A shirting material which has been dyed with

0.5 per cent. of Cibalone Blue GCD (Schultz, Farbstofftabellen, 7th edition, 1931, No. 1,234) and is unsuitable for making up into clothing owing to unlevel dyeing, is treated in a jigger for 5 half-an-hour at 60° C. with a solution containing per liter 15 cc. of an aqueous solution of sodium hydroxide of 36° Bé., 5 grams of sodium hydrosulfite and 0.2 gram of the product prepared by sulfonating a mixture of 25 per cent. of N-methyl- $\mu$ -heptadecylbenzimidazole and 75 per cent. of 10 N:N-methyl-ethyl- $\mu$ -heptadecylbenzimidazolium chloride.

There is obtained in this manner a piece material which is dyed uniformly throughout and is 15 suitable for making up into clothing. Similar results are obtained when using other quantitative proportions than indicated in the first paragraph of this example, e. g. 30 to 70, 50 to 50 or 70 to 30.

## 20

*Example 4*  
A padding bath is prepared with 50 grams of Cibalone Violet 2R double paste (Schultz, Farbstofftabellen, 7th edition, 1931, No. 1,265) and 5 grams of the product of the sulfonation of a mixture of 25 per cent. of N-methyl- $\mu$ -heptadecylbenzimidazole and 75 per cent. of N:N-methyl-ethyl- $\mu$ -heptadecylbenzimidazolium chloride.

A linen fabric is passed repeatedly through the bath and intermediately between squeezing rollers. The dyeing is then developed in a jigger by 30 treating the fabric at 60° C. with a liquor containing per liter 16 cc. of sodium hydroxide solution of 36° Bé. and 2 grams of sodium hydrosulfite.

The fabric is thus dyed very evenly and is well 35 through-dyed. Similar results are obtained when using other quantitative proportions than indicated in the first paragraph of this example, e. g. 30 to 70, 50 to 50 or 70 to 30.

## 40

*Example 5*  
For dyeing 100 kilos of loose wool, a dye-bath of about 1000 liters and having a temperature of 55° C. is prepared with the aid of 500 grams of glue, 500 cc. of ammonia of specific gravity 0.9, 300 45 grams of sodium hydrosulfite and 500 grams of the sodium salt of sulfonated N-methyl- $\mu$ -heptadecylbenzimidazole. Thereupon there are added 2.5 kilos of Ciba Blue 2B (Schultz, Farbstofftabellen, 7th edition, No. 1,314), which have previously 50 been vatted in the customary manner.

The addition of the sulfonated benzimidazole derivative has the effect of retarding appreciably absorption of the dyestuff so that the whole batch is dyed much more evenly than in the absence 55 of such a derivative. The benzimidazole-sulfonic acids alkylated at the N-atom mentioned at the end of Example 1 behave similarly.

## 60

*Example 6*  
For dyeing mercerized bead yarn there is added to the dye-bath, containing 0.5 per cent. of Cibalone Violet 2R (Schultz, Farbstofftabellen, 7th edition, No. 1,265) or 0.5 per cent. of Cibalone Blue 3G (Schultz, Farbstofftabellen, 7th 65 edition, No. 1,279), vatted in the customary manner; the sodium salt of sulfonated N-methyl-N-benzyl- $\mu$ -heptadecylbenzimidazolium-chloride in a quantity amounting to 0.2 gram per liter of the dye-bath. The dyestuff is absorbed substantially more slowly than in the absence of this 70 addition and in consequence the material is dyed more evenly and is better through-dyed.

## Example 7

Cotton piece goods are dyed in a jigger with an alkaline hydrosulfite bath containing 0.5 per cent. of Cibalone Violet 2R (Schultz, Farbstofftabellen, 7th edition, 1931, No. 1,265), with the 5 addition, per liter of dye-bath, of 0.5 gram of the sodium salt of the product prepared by sulfonating the quaternary hexadecyl-phenyl-dimethyl-ammonium-methylsulfate. The dyeings 10 are appreciably more level than those obtained without this addition.

A like effect is obtained if instead of the aforesaid addition there is added, per liter of dye-bath, 1 gram of the sodium salt of sulfonated 15 N-methyl-hexadecyl-aniline, or 2 grams of the sodium salt of sulfonated hexadecyl-aniline.

## Example 8

Cotton drapery material is dyed by means of 20 20 per cent. of Pyrogene Indigo (Schultz, Farbstofftabellen, 7th edition, No. 1,110) in a bath containing besides the usual additions, 0.3 gram per liter of the sodium salt of N-methyl-hep-25 tacylbenzimidazol-sulfonic acid.

Owing to the addition of this substance the dyestuff is appreciably more slowly absorbed; the dyeing is much more level and the material is better through-dyed. Furthermore, the dyeing shows no tendency towards bronzing.

What we claim is:—

1. Baths used for treating textile materials containing cellulose, which baths are characterized by a content of alkali, a reducing agent, and 35 a sulfonated benzimidazole substituted at the  $\mu$ -carbon atom by an aliphatic chain having at least 8 carbon atoms.

2. Baths used for treating textile materials containing cellulose, which baths are characterized by a content of alkali, hydrosulfite, and a 40 sulfonated benzimidazole substituted at the  $\mu$ -carbon atom by an aliphatic chain having at least 8 carbon atoms.

3. Baths used for treating textile materials containing cellulose, which baths are characterized by a content of alkali, hydrosulfite, and a sulfonated benzimidazole substituted at the 45  $\mu$ -carbon atom by the heptadecyl radical.

4. Baths used for treating textile materials containing cellulose, which baths are characterized by a content of alkali, hydrosulfite, and a sulfonated benzimidazole substituted at the  $\mu$ -carbon atom by the heptadecyl radical and at 50 least one nitrogen atom by an alkyl radical containing not more than 4 carbon atoms.

5. Baths used for treating textile materials containing cellulose, which baths are characterized by a content of alkali, hydrosulfite and an alkali salt of the sulfonated N-methyl- $\mu$ -hep-55 tacylbenzimidazolium chloride.

6. Baths used for treating textile materials containing cellulose, which baths are characterized by a content of alkali, hydrosulfite and an alkali salt of a sulfonated mixture of N-methyl- $\mu$ -heptadecylbenzimidazole and N-methyl-N'-65 ethyl- $\mu$ -heptadecylbenzimidazolium chloride.

CHARLES GRAENACHER.  
FRANZ ACKERMANN.  
ALBERT LANDOLT.  
WILHELM GEIGY.